

## UNITED STATES PATENT OFFICE

2,322,025

## CONVERSION OF HYDROCARBONS

Vladimir N. Ipatieff and Aristid V. Grosse, Chicago, Ill., assignors to Universal Oil Products Company, Chicago, Ill., a corporation of Delaware

No Drawing. Application April 3, 1939,  
Serial No. 265,776

4 Claims. (CL. 260—683)

This application is a continuation-in-part of our co-pending application Serial No. 28,670 filed June 27, 1935.

This invention relates particularly to conversion reactions among lower molecular weight hydrocarbons of an olefinic and paraffinic character which are normally gaseous at ordinary temperatures and pressures.

More specifically the invention is concerned with the practical application of a new type of reaction involving catalysts in the transfer of combined hydrogen from one type of hydrocarbon to another. The process may involve the interaction of hydrocarbons in synthetic mixtures and is particularly applicable in the case of the hydrocarbon gas mixtures produced incidental to oil cracking operations.

In the cracking of heavy hydrocarbon fractions representing residua and the heavier distillates from petroleum with the primary object of producing maximum yields of low boiling gasoline hydrocarbons there is invariably produced a considerable amount of normally gaseous hydrocarbons which at the present time are utilized principally as fuel although they contain large percentages of reactive olefin hydrocarbons in contrast to the analogous mixtures produced in connection with the production and the straight run distillation of the original petroleum. Cracked gases contain varying percentages of the compounds shown in the following table:

|           |                  |
|-----------|------------------|
| Hydrogen  | Butanes          |
| Methane   | Butylenes        |
| Ethane    | Pentanes         |
| Ethylene  | Amylenes         |
| Propane   | Hydrogen sulfide |
| Propylene |                  |

Inasmuch as the gaseous products of the cracking reaction may at times amount to from 10 to 15% by weight of the original oil cracked, it is obviously a matter of some importance to make the most efficient use of the gaseous by-products.

The so-called natural gases produced alone or in conjunction with the production or primary distillation of petroleum comprise the paraffin hydrocarbons indicated in the above table, being substantially devoid of hydrogen and olefins. As will be later developed these gases may also constitute a source of starting material for the present process. The olefinic constituents in cracked hydrocarbon gas mixtures have been employed to some extent as starting material for the manufacture of alcohols by treatment with acids such as sulfuric followed by the hydrolysis of the acid

esters and as a basis for the manufacture of halogen derivatives and certain secondary chemical products. However, from the petroleum refiners' standpoint greater interest attaches to the reconversion of as much as possible of the gaseous products of straight run distillation and cracking into gasoline, since the average refinery has a superabundance of fuel of all kinds and frequently the fixed gas production is in excess of the total refinery requirements, including steam generation. The marketing of the excess gas as domestic and industrial fuel has been undertaken to some extent but in this case the demand fluctuates with the seasons and the storage and handling of the gases require special installations of gas holders, etc.

Recent investigations of the possibilities of utilizing the olefinic constituents of cracked gases have considered the possibility of condensing or polymerizing the olefins to form polymers boiling within the normal range of present day motor fuels, that is, from about 100 to 400° F., since the dimers and a considerable number of the trimers and the mixed polymers producible from the olefinic constituents of the gases boil within this range. Development work has been divided along the lines of either straight heat treatment or catalytic polymerization. In the former case the yields are inclined to be low and the process requires very careful manipulation so that in general it may be said that the industry is in favor of the catalytic processes when dealing with cracked gas mixtures. These processes have employed numerous catalytic materials including mineral acids such as sulfuric and phosphoric acid alone or with spacing or carrying agents and also certain metallic salts having polymerizing properties such as, for example, aluminum chloride, zinc chloride, etc. Some attempts have been made to utilize solid contact materials of the nature of fuller's earth but without any signal success.

In catalytic polymerization processes the principal effects are observed in connection with the olefins containing more than 2 carbon atoms, to wit, propylene, alpha and beta butenes and isobutylene, the readiness with which these polymerize being inverse to the order in which they were just given. In regard to ethylene this compound is so much more difficult to polymerize than the higher gaseous olefins that in most cases it is substantially unaffected under conditions which readily polymerize propylene and the butylenes. If more severe conditions are employed the ethylene tends to polymerize more to form

higher boiling polymers than those of gasoline boiling range although in certain instances it is evident that ethylene undergoes some condensation reactions with the other olefins of higher molecular weight. The polymers produced by the combination of gasoline olefin molecules are of high antiknock value and relatively stable and thus are very desirable blending fluids for raising the octane number of straight run gasolines.

In present day gas utilization processes, the paraffins are of the least value since as such they are unreactive and not capable of forming liquids except in small amounts under severe conditions of pyrolysis, which are seldom economical. The conversion of the propanes and the butanes in cracked or natural gases into olefins which are readily polymerizable is an important feature of the present invention, which stands as an improvement in the art of utilizing the gaseous by-products encountered both in the straight and in the destructive distillation of petroleum.

In one specific embodiment the present invention comprises the production of olefins of more than 2 carbon atoms by reacting the corresponding paraffins with ethylene in the presence of catalysts particularly adapted to accelerating the reactions.

The type of reactions with which the present process is concerned is exemplified by the two following equations which show the interaction of ethylene with 3 and 4 carbon atom paraffin hydrocarbons respectively, whereby ethane and 3 and 4 carbon atom olefins are produced.



We have found that, in the presence of suitable catalysts which will be presently described in detail, it is possible to effect an almost quantitative transfer of hydrogen from paraffins to ethylene so that it becomes saturated and in effect its unsaturation is transferred to the compounds of higher molecular weight to yield olefins. The value of such catalyzed reactions is at once apparent in that the resulting olefins are readily polymerized by various types of catalysts to form gasoline boiling range polymers of superior antiknock value and generally stable characteristics. It is further evident that by this type of reaction increased proportions of refinery gases including straight run and cracked gases are made available for the production of gasoline. The ethane produced in the above equations may be dehydrogenated in the presence of the same general types of catalysts suited to the above reactions and reused almost indefinitely so that the process is substantially cyclic and may be operated at a high efficiency.

The progress of the above equations depends largely upon the preferential affinity of ethylene for hydrogen in the presence of the preferred catalysts. The types of catalysts which may be employed for furthering and promoting the extent of the above type of reactions are certain of those which have been found to be effective in so-called dehydrogenation reactions. In other words, such catalysts have value in promoting the splitting off of a molecule of hydrogen from a paraffin to produce the corresponding olefin and we have now determined that some of the same materials are particularly effective in transferring hydrogen from paraffins to ethylene, the ethylene acting as an "acceptor" of the released

hydrogen, and enabling the reactions to proceed rapidly to equilibrium.

The preferred catalysts in accordance with the present invention consists of alumina (preferably activated) supporting certain alkaline earth metal salts and the oxides of the heavy metals chromium, molybdenum, and vanadium. Alternatively, the chromates and molybdates of beryllium, magnesium, calcium, barium, strontium, and zinc may be employed although as a rule the preferred catalyst composites comprise alumina plus oxides of chromium, molybdenum, and vanadium. The materials added to the alumina to increase its catalytic activity are usually less than 25% by weight of the total composites although it is not intended to limit the invention to this particular range of concentration.

Aluminum oxide suitable as the base material for the manufacture of catalysts for the process may be obtained from some natural aluminum oxide minerals or ores such as bauxite, or prepared by precipitation of aluminum hydroxide from solutions of aluminum sulfate, nitrate, chloride, or different other salts, and dehydration of the precipitate of aluminum hydroxide by heat. Usually it is desirable and advantageous to further treat it with air or other gases, or by other means to activate it prior to use.

Three hydrated oxides of aluminum occur in nature, to wit, hydrargillite or gibbsite having the formula  $\text{Al}_2\text{O}_3 \cdot 3\text{H}_2\text{O}$ , bauxite having the formula  $\text{Al}_2\text{O}_3 \cdot 2\text{H}_2\text{O}$ , and diasporite having the formula  $\text{Al}_2\text{O}_3 \cdot \text{H}_2\text{O}$ . Of these minerals the corresponding oxides from the trihydrated and dihydrated minerals are suitable for the manufacture of alumina for the present type of catalysts and these materials have furnished types of activated alumina which are entirely satisfactory as supports for the preferred catalytic substances. Precipitated trihydrates can also be dehydrated at moderately elevated temperatures to form satisfactory alumina supports.

It is best practice in the final steps of preparing substantially anhydrous aluminum oxides for use as catalyst supports to ignite them for some time at temperatures within the approximate range of from 600-650° C. This does not correspond to complete dehydration of the hydrated oxides but gives supporting materials of good strength and porosity so that they are able to resist for a long period of time the deteriorating effects of the service and regeneration periods to which they are subjected.

In applying the process to the production of readily polymerizable olefins e. g. propene and butene it is only necessary to pass proportioned mixtures of propane or butanes with ethylene through beds of selected granular catalytic material which is contained in treating chambers as filler. Temperatures of from 150 to 700° C. may be employed depending upon the efficacy of the particular catalyst used and atmospheric or moderately superatmospheric pressures are usually all that are required. The catalysts are most selective in their reactions at the lower temperatures but the reaction velocity increases with increase in temperatures and therefore a balance will be struck in practice between these two factors.

After the reactions are completed in any given instance the gas mixture containing the higher molecular weight olefins may be contacted directly with suitable polymerizing catalysts such as, for example, the so-called solid phosphoric acid catalysts, to remove the olefins and the eth-

ylene necessary for further reaction may be regenerated from the residual ethane by dehydrogenating it using the same general types of catalysts employed in the main reactions.

Best results in regard to olefin production are usually obtained when a given paraffin is reacted with its molecular equivalent of ethylene. However, in the case of certain cracked gas mixtures which contain the higher gaseous paraffins and relatively large percentages of ethylene in comparison with the amounts of higher olefins, they may be subjected to contact with dehydrogenating catalysts as they are produced prior to the subjection of the gas mixture to the action of polymerizing catalysts to produce the desired liquid polymers for blending with inferior knock rating gasolines.

In the case of stabilizer refluxes operated in conjunction with oil cracking plants it is usually good practice to polymerize the 3 and 4 carbon atom olefins by the use of effective catalysts and then add regulated amounts of ethylene to the gas mixture for the conversion of the residual 3 and 4 carbon atom paraffins to their corresponding olefins by reactions of the present character.

The following example is given to illustrate the character of the results obtainable by the use of the present process although it is not to be looked upon in a limiting sense as regards the scope of the invention, since other data are available.

A mixture of ethylene and normal butane was passed at atmospheric pressure and a temperature of 450° C. over a catalyst comprising alumina oxide and having deposited thereon about 5% of chromium trioxide. The composition of the inlet and exit gases is given below:

|                | Inlet gas | Exit gas |
|----------------|-----------|----------|
|                | Per cent  | Per cent |
| Ethylene.....  | 25        | 2        |
| n-Butane.....  | 75        | 56       |
| Ethane.....    | 0         | 20       |
| Butylenes..... | 0         | 20       |
| Hydrogen.....  | 0         | 2        |
|                | 100       | 100      |

The analysis indicates that the ethylene was

converted to ethane with a relatively high efficiency, that there was very little hydrogen actually released as such in the course of the reactions and that practically all the conversion products arising from the n-butane were butylenes. These conditions generally obtain up to equi-molecular mixtures of butane and ethylene, though the efficiency of the desired reaction drops off slightly and somewhat larger quantities of free hydrogen appear. Thus with any given paraffin which is to be converted into an olefin by the present type of reaction, a proportion of ethylene to paraffin would be reached corresponding to maximum efficiency when utilizing a recycling operation so that the unconverted paraffin is returned for further catalytic treatment and dehydrogenation.

The foregoing descriptive section shows at once the novelty and utility of the present invention and the numerical data presented are sufficient for its commercial value. However, neither section is intended to be unduly limiting.

We claim as our invention:

1. A process which comprises reacting a paraffin containing more than two carbon atoms with ethylene in the presence of a catalyst effective in transferring hydrogen from the paraffin to the ethylene, thereby forming ethane and an olefin of more than two carbon atoms, subjecting the admixed ethane and olefin to polymerization to convert the latter to liquid and thereby separate it from the ethane, dehydrogenating the separated ethane and supplying resultant ethylene to the first-mentioned step of the process.

2. The process as defined in claim 1 further characterized in that said catalyst comprises alumina supporting an oxygen-containing compound of chromium.

3. The process as defined in claim 1 further characterized in that said catalyst comprises alumina supporting an oxygen-containing compound of molybdenum.

4. The process as defined in claim 1 further characterized in that said catalyst comprises alumina supporting an oxygen-containing compound of vanadium.

VLADIMIR N. IPATIEFF.  
ARISTID V. GROSSE.